



US006044893A

# United States Patent [19]

Taniguchi et al.

[11] Patent Number: 6,044,893

[45] Date of Patent: Apr. 4, 2000

[54] **METHOD AND APPARATUS FOR PRODUCTION OF AMORPHOUS ALLOY ARTICLE FORMED BY METAL MOLD CASTING UNDER PRESSURE**

[75] Inventors: **Takeshi Taniguchi; Junichi Nagahora**, both of Sendai, Japan

[73] Assignee: **YKK Corporation**, Tokyo, Japan

[21] Appl. No.: **09/066,052**

[22] Filed: **Apr. 27, 1998**

[30] Foreign Application Priority Data

May 1, 1997 [JP] Japan ..... 9-126229

[51] Int. Cl.<sup>7</sup> ..... B22D 18/06; B22D 31/00

[52] U.S. Cl. ..... 164/70.1; 164/63; 164/113

[58] Field of Search ..... 164/113, 63, 70.1, 164/69.1

[56] References Cited

U.S. PATENT DOCUMENTS

5,032,196 7/1991 Masumoto et al. ....  
5,579,825 12/1996 Shibata et al. ..... 164/113  
5,711,363 1/1998 Scruggs et al. ..... 164/113

FOREIGN PATENT DOCUMENTS

0 710 515 5/1996 European Pat. Off. ....  
1 805 933 6/1969 Germany ....  
41 06 605 9/1991 Germany ....  
58-084659 5/1983 Japan .... 164/113  
58-159965 9/1983 Japan ..... 164/113  
59-133962 8/1984 Japan ..... 164/63  
60-076264 4/1985 Japan .

60-154861 8/1985 Japan .  
63-062838 3/1988 Japan .  
63-278636 11/1988 Japan .  
03165961 7/1991 Japan .  
4-172163 6/1992 Japan ..... 164/113  
8-199318 8/1996 Japan .  
WO 93/11895 6/1993 WIPO ..... 164/63

Primary Examiner—Kuang Y. Lin

Attorney, Agent, or Firm—Finnegan, Henderson, Farabow, Garrett & Dunner, L.L.P.

[57] ABSTRACT

A method and apparatus for producing a formed article of amorphous alloy by a simple process are disclosed. A molding apparatus comprises a forced cooling casting mold which is provided with a sprue and at least one molding cavity communicating with the sprue and further with a cutting member disposed in the casting mold movably in the direction of the sprue, a melting vessel movable in the direction of the sprue, and a molten metal transferring member disposed slidably in the melting vessel or the molding cavity of the casting mold. A formed article of amorphous alloy is obtained by melting an alloying material in the vessel, forcibly transferring the resultant molten alloy into the molding cavity by means of the molten metal transferring member and meanwhile exerting pressure on the molten alloy, rapidly cooling and solidifying the molten alloy in the casting mold thereby conferring amorphousness on the alloy and meanwhile gradually cooling and solidifying the molten alloy in the part of the sprue of the casting mold thereby crystallizing the alloy in that part, cutting the part which has been embrittled by the crystallization by means of the cutting member, and thereafter separating the melting vessel from the casting mold.

9 Claims, 10 Drawing Sheets



FIG. 1



FIG. 2



FIG. 3



FIG. 4



FIG. 5



FIG. 6



FIG. 7



FIG. 8



FIG. 9



FIG. 10

45



FIG. 11



## 1

**METHOD AND APPARATUS FOR  
PRODUCTION OF AMORPHOUS ALLOY  
ARTICLE FORMED BY METAL MOLD  
CASTING UNDER PRESSURE**

**BACKGROUND OF THE INVENTION**

**1. Field of the Invention**

This invention relates to a method and apparatus for the production of an amorphous alloy article formed by metal mold casting under pressure.

**2. Description of the Prior Art**

The single roll method, twin roll method, gas atomizing method, etc. are adopted for the production of amorphous alloy because this production generally necessitates a high cooling rate falling in the approximate range of  $10^4$ – $10^6$  K/s. The products obtained by such methods are limited in shape to ribbons of foil, fine wires, and particles. This fact constitutes itself a factor for rigidly limiting the field of applications found for amorphous alloy.

Feasibility studies are under way, therefore, regarding a method of producing a formed article of amorphous alloy with a large thickness by shaping an amorphous alloy prepared in the form of powder by some means such as extrusion or impact compression at a temperature not exceeding the crystallization temperature of the alloy. The production by this method, however, requires complicated steps such as sieving the powder, degassing the prepared powder, and preforming the powder prior to the main forming and calls for expensive facilities as well. This method, therefore, is at a disadvantage in inevitably furnishing only expensive products.

As a means for producing a formed article of amorphous alloy by a simple process unlike such powder molding process, published Japanese Patent Application, KOKAI (Early Publication) No. 8-199,318 discloses a method for the production of a rod or tube of a Zr-based amorphous alloy by disposing a forced cooling casting mold having a molding cavity fitted with a molten metal transfer tool on the bottom of a hearth opened on the top side, melting a zirconium alloy containing an element capable of conferring amorphousness on the alloy in the hearth, then extracting the molten metal transfer tool downwardly thereby transferring the melt of the zirconium alloy into the forced cooling casting mold, and rapidly cooling and solidifying the melt of zirconium alloy in the forced cooling casting mold thereby conferring amorphousness on the zirconium alloy.

According to the method described above, however, the cast products have their shapes limited to rods or tubes because their shapes are restricted by the shape of the molten metal transfer tool and the method of extraction of this tool. Further, this method is incapable of substantially pressing the molten alloy because the transfer of the molten alloy is induced simply by the extraction of the molten metal transfer tool. The method, therefore, incurs difficulty in yielding formed articles which are delicate or complicate in shape and the products thereof have room for improvement in terms of denseness and mechanical properties.

**SUMMARY OF THE INVENTION**

It is, therefore, an object of the present invention to provide a method which, owing to the combination of a technique based on the conventional metal mold casting process with the quality of an amorphous alloy exhibiting a glass transition region, allows a formed article of amorphous alloy satisfying a stated shape, dimensional accuracy, and

## 2

surface quality despite complexity or delicateness of shape to be mass-produced with high efficiency by a simple process and, therefore, enables the production of even a precision machined article to omit or diminish markedly such machining steps as grinding and consequently provide an inexpensive formed article of amorphous alloy excelling in durability, strength, and resistance to impact.

It is another object of the present invention to provide an apparatus of relatively simple construction which fits the production of such formed article of amorphous alloy as mentioned above.

To accomplish the objects described above, according to the first aspect of the present invention, there is provided a method for the production of a formed article of amorphous alloy, which method is characterized by comprising melting an alloying material capable of yielding an amorphous alloy in a melting vessel, forcibly transferring the resultant molten alloy into a forced cooling casting mold provided with at least one molding cavity and meanwhile exerting pressure on the molten alloy, and rapidly cooling and solidifying the molten alloy in the forced cooling casting mold to confer amorphousness on the alloy thereby obtaining a formed article of an alloy containing an amorphous phase.

In a preferred embodiment, the steps mentioned above are carried out in a vacuum or under an atmosphere of inert gas. In another preferred embodiment, the formed article of an alloy containing an amorphous phase is obtained by melting an alloying material capable of yielding an amorphous alloy in a melting vessel having an upper open end, forcibly transferring the resultant molten alloy into the forced cooling casting mold provided with at least one molding cavity via a sprue thereof and meanwhile exerting pressure on the molten alloy, rapidly cooling and solidifying the molten alloy in the forced cooling casting mold thereby conferring amorphousness on the alloy and meanwhile gradually cooling and solidifying the molten alloy in the part of the sprue of the forced cooling casting mold thereby crystallizing the alloy in that part, cutting the part which has been embrittled by the crystallization, and thereafter separating the melting vessel from the forced cooling casting mold.

The forced transfer of the molten alloy into the forced cooling casting mold can be preferably effected by a method which comprises disposing movably in the melting vessel a molten metal transferring member adapted to effect forced transfer of the molten alloy and forcibly transferring the molten alloy held in the melting vessel into the forced cooling casting mold and meanwhile exerting pressure on the molten alloy now filling the molding cavity of the forced cooling casting mold by means of the molten metal transferring member.

Another method available for this purpose comprises disposing preparatorily the molten metal transferring member movably in the forced cooling casting mold and moving the molten metal transferring member so as to generate negative pressure inside the molding cavity and consequently induce forced transfer of the molten alloy into the molding cavity. In one preferred embodiment of this method, the molten metal transferring member to be used is furnished with a cross section conforming to that of the molding cavity of the forced cooling casting mold and slidably disposed in the molding cavity. The exertion of pressure on the molten alloy filling the molding cavity is attained by applying a pressurized gas to the molten alloy via the sprue.

In any of the methods described above, as the alloying material mentioned above, an alloy which possesses a com-

position represented by the following general formula and which is capable of yielding an amorphous alloy having a glass transition region of a temperature width of not less than 30 K is advantageously used.



wherein X represents either or both of the two elements, Zr and Hf, M represents at least one element selected from the group consisting of Mn, Fe, Co, Ni, and Cu, and a, b, and c represent such atomic percentages as respectively satisfy  $25 \leq a \leq 85$ ,  $5 \leq b \leq 70$ , and  $0 < c \leq 35$ . This amorphous alloy contains an amorphous phase in a volumetric ratio of at least 50%.

In accordance with the second aspect of the present invention, there is provided an apparatus which can be suitably used for producing such formed article of amorphous alloy as mentioned above.

The first embodiment of the apparatus of the present invention for the production of the formed article of amorphous alloy is characterized by comprising a forced cooling casting mold which is provided in the lower part thereof with a sprue and in the inner part thereof with at least one molding cavity communicating with the sprue through the medium of a runner and further provided with a cutting member disposed in the casting mold movably in the direction of the sprue; and a melting vessel disposed under the casting mold movably in the direction of the sprue, which vessel is provided with a raw material accommodating hole having an upper open end and a molten metal transferring member disposed slidably in the raw material accommodating hole.

The second embodiment of the apparatus of the present invention is characterized by comprising a vertically movable melting vessel having a lower open end; and a forced cooling casting mold disposed under the melting vessel, which casting mold is provided with a closable sprue and at least one molding cavity adapted to establish, when the casting mold is in close contact with the lower part of the melting vessel, communication with the sprue through the medium of a runner and further with a molten metal transferring member disposed slidably in the molding cavity and a cutting member disposed in the casting mold and movable in the direction of the sprue.

Preferably in either of the embodiments described above, a closing member which is movable perpendicularly to the direction of the movement of the cutting member is interposed between the cutting member and the runner and the peripheral all portion of the sprue and/or the closing member is made of an insulating material. Further, the forced cooling casting mold and the melting vessel mentioned above are preferably installed in a vacuum or in an atmosphere of inert gas.

#### BRIEF DESCRIPTION OF THE DRAWINGS

Other objects, features, and advantages of the invention will become apparent from the following description taken together with the drawings, in which:

FIG. 1 is a fragmentary cross-sectional view schematically illustrating one example of the apparatus of the present invention for molding a tube;

FIG. 2 is a fragmentary cross-sectional view illustrating the essential part of the apparatus shown in FIG. 1 during the injection of molten alloy;

FIG. 3 is a fragmentary cross-sectional view illustrating the essential part of the apparatus shown in FIG. 1 after the molten metal has solidified;

FIG. 4 is a fragmentary cross-sectional view illustrating the essential part of the apparatus shown in FIG. 1 after the solidified material has been cut;

FIG. 5 is a fragmentary cross-sectional view illustrating the essential part of the apparatus shown in FIG. 1 during the reinjection of molten alloy;

FIG. 6 is a perspective view illustrating a cast article produced by the apparatus shown in FIG. 1;

FIG. 7 is a plan view of the cast article shown in FIG. 6;

FIG. 8 is a plan view illustrating another example of cast article;

FIG. 9 is a fragmentary cross-sectional view illustrating schematically one example of the forced cooling casting mold for the formation of a toothed wheel according to the present invention;

FIG. 10 is a perspective view illustrating a toothed wheel produced by the forced cooling casting mold shown in FIG. 9; and

FIG. 11 is a fragmentary cross-sectional view illustrating schematically another example of the apparatus for the formation of a tube according to the present invention.

#### DETAILED DESCRIPTION OF THE INVENTION

The production of a formed article of amorphous alloy according to the present invention is characterized, as described above, by comprising melting an alloying material capable of yielding an amorphous alloy in a melting vessel, forcibly transferring the resultant molten alloy into a forced cooling casting mold provided with a cavity for molding a product and meanwhile exerting pressure on the molten alloy, and rapidly cooling and solidifying the molten alloy in the casting mold to obtain a formed article of an alloy containing an amorphous phase. In this case, the forced transfer of the molten alloy into the molding cavity of the forced cooling casting mold can be attained by a method which comprises causing a molten metal transferring member disposed slidably in the melting vessel to be actuated by a hydraulic or pneumatic cylinder, for example, thereby inducing forced transfer of the molten alloy held in the vessel into the molding cavity of the casting mold and meanwhile pressing the molten alloy filling in the molding cavity or a method which comprises having the molten metal transferring member preparatorily disposed slidably inside the molding cavity of the casting mold, moving the molten metal transferring member so as to induce generation of negative pressure in the molding cavity and effecting forced transfer of the molten alloy into the molding cavity and meanwhile adding a gas pressure to the melting vessel.

These methods, owing to the fact that the molten alloy which is placed in the molding cavity of the forced cooling casting mold is held in a pressed state, enable a formed article even in a complicated shape or a delicate shape to be mass-produced efficiently and therefore inexpensively by a simple process. Thus, the resultant formed article faithfully reproduces the contour of the molding cavity with high dimensional accuracy and acquires high denseness and smooth surface.

Further by carrying out the component steps of the process mentioned above in a vacuum or under an atmosphere of inert gas, the molten alloy can be prevented from producing an oxide film and the formed article of amorphous alloy can be manufactured in highly satisfactory quality. For the purpose of preventing the molten metal from producing an oxide film, it is preferable to have the apparatus in its entirety disposed in a vacuum or in an atmosphere of inert gas such as Ar gas or to sweep at least the upper part of the melting vessel exposing the molten alloy to the ambient air with a stream of inert gas.

In the apparatus of the present invention for the production of a formed article of amorphous alloy, a cutting member is disposed in the forced cooling casting mold so as to be movable in the direction of a sprue of the casting mold and, after completion of the solidification of the molten alloy, enabled to sever the hardened portion persisting in the sprue or additionally inside the melting vessel from the cast article placed and hardened in the casting mold and allow easy separation of the melting vessel and the casting mold subsequently to completion of the casting step. As a result, the next casting step can be carried out smoothly with improved operational efficiency.

Preferably, the peripheral wall part of the sprue and/or a closing member interposed between the cutting member and a runner of the casting mold and allowed to move perpendicularly to the direction of transfer of the cutting member are made of an insulating material so that these parts may cool at a lower rate than the interior of the molding cavity. By insulating the sprue as described above, the flow of the molten alloy is smoothed and the molten alloy poured into the molding cavity of the casting mold is rapidly cooled and solidified and allowed to assume amorphousness. Since the molten alloy lodged in the part of the sprue is slowly cooled and solidified and consequently crystallized, the part which is embrittled by this crystallization can be cut easily.

The material for the formed article of the present invention does not need to be limited to any particular substance but may be any of the materials which are capable at all of furnishing a product formed substantially of amorphous alloy. Among other materials answering this description, the Zr—TM—Al and Hf—TM—Al (TM: transition metal) amorphous alloys represented by the general formula mentioned above and having very wide differences between the glass transition temperature (Tg) and the crystallization temperature (Tx) exhibit high strength and high corrosion resistance, possess wide super-cooled liquid ranges (glass transition ranges),  $\Delta T_x = T_x - T_g$ , of not less than 30 K, and extremely wide supercooled liquid ranges of not less than 60 K in the case of the Zr—TM—Al amorphous alloys. In the above temperature ranges, these amorphous alloys manifest very satisfactory workability owing to viscous flow even at such low stress not more than some tens MPa. They are characterized by being produced easily and very stably as evinced by the fact that they are enabled to furnish an amorphous bulk material even by a casting method using a cooling rate of the order of some tens K/s. The aforementioned Zr—TM—Al and Hf—TM—Al amorphous alloys are disclosed in U.S. Pat. No. 5,032,196 issued Jul. 16, 1991 to Masumoto et al., the teachings of which are hereby incorporated by reference. By the metal mold casting from melt and by the molding process utilizing the viscous flow resorting to the glass transition range as well, these alloys produce amorphous materials and permit very faithful reproduction of the shape and size of a molding cavity of a metal mold.

The Zr—TM—Al and Hf—TM—Al amorphous alloys to be used in the present invention possess very large range of  $\Delta T_x$ , though variable with the composition of alloy and the method of determination. The  $Zr_{60}Al_{15}Co_{2.5}Ni_{7.5}Cu_{15}$  alloy (Tg: 652 K, Tx: 768 K), for example, has such an extremely wide  $\Delta T_x$  as 116 K. It also offers very satisfactory resistance to oxidation such that it is hardly oxidized even when it is heated in the air up to the high temperature of Tg. The Vickers hardness (Hv) of this alloy at temperatures from room temperature through the neighborhood of Tg is 460 (DPN), the tensile strength thereof is 1,600 MPa, and the bending strength thereof is up to 3,000 MPa. The thermal

expansion coefficient,  $\alpha$  of this alloy from room temperature through the neighborhood of Tg is as small as  $1 \times 10^{-5}/K$ , the Young's modulus thereof is 91 GPa, and the elastic limit thereof in a compressed state exceeds 4–5%. Further, the toughness of the alloy is high such that the Charpy impact value falls in the range of 6–7 J/cm<sup>2</sup>. This alloy, while exhibiting such properties of very high strength as mentioned above, has the flow stress thereof lowered to the neighborhood of 10 MPa when it is heated up to the glass transition range thereof. This alloy, therefore, is characterized by being worked very easily and being manufactured with low stress into minute parts and high-precision parts complicated in shape. Moreover, owing to the properties of the so-called glass (amorphous) substance, this alloy is characterized by allowing manufacture of formed (deformed) articles with surfaces of extremely high smoothness and having substantially no possibility of forming a step which would arise when a slip band appeared on the surface as during the deformation of a crystalline alloy.

Generally, an amorphous alloy begins to crystallize when it is heated to the glass transition range thereof and retained therein for a long time. In contrast, the aforementioned alloys which possess such a wide  $\Delta T_x$  range as mentioned above enjoy a stable amorphous phase and, when kept at a temperature properly selected in the  $\Delta T_x$  range, avoid producing any crystal for a duration up to about two hours. The user of these alloys, therefore, does not need to feel any anxiety about the occurrence of crystallization during the standard molding process.

The aforementioned alloys manifest these properties unreservedly during the course of transformation thereof from the molten state to the solid state. Generally, the manufacture of an amorphous alloy requires rapid cooling. In contrast, the aforementioned alloys allow easy production of a bulk material of a single amorphous phase from a melt by the cooling which is effected at a rate of about 10 K/s. The solid bulk material consequently formed also has a very smooth surface. The alloys have transferability such that even a scratch of the order of microns inflicted by the polishing work on the surface of a metal mold is faithfully reproduced.

When the aforementioned alloys are adopted as the alloying material, therefore, the metal mold to be used for producing the formed article is only required to have the surface thereof adjusted to fulfill the surface quality expected of the article because the article produced faithfully reproduces the surface quality of the metal mold. In the conventional metal mold casting method, therefore, these alloys allow the steps for adjusting the size and the surface roughness of the molded article to be omitted or diminished.

The characteristics of the aforementioned amorphous alloys which combine high tensile strength and high bending strength, satisfactory Young's modulus, high elastic limit, high impact resistance, fine surface smoothness, and castability or workability of high precision can be advantageously applied to formed articles in various fields such as, for example, precision parts represented by ferrules and sleeves in optical fiber connectors, toothed wheels, and micromachines.

The amorphous alloys represented by the general formula,  $X_aM_bAl_c$ , mentioned above manifest the same characteristics as mentioned above even when they incorporate such elements as Ti, C, B, Ge, or Bi at a ratio of not more than 5 atomic %.

Now, the present invention will be described more specifically below with reference to embodiments illustrated in the drawings annexed hereto.

FIG. 1 schematically illustrates the construction of one example of the apparatus for producing a tube of amorphous alloy by the method of the present invention.

A forced cooling casting mold **10** is a split mold composed of an upper mold **11** and a lower mold **20**. The upper mold **11** has a pair of molding cavities **12a** and **12b** formed therein and adapted to define the outside dimension of a cast article. These cavities **12a** and **12b** intercommunicate through the medium of a runner **13** such that the molten metal flows through the leading ends of such parts **14a** and **14b** of the runner as half encircle the peripheries of the cavities **12a** and **12b** at a prescribed distance into the cavities **12a** and **12b**. In the upper mold **11**, air vents **15a** and **15b** are formed as extended from the upper ends of the cavities **11a** and **11b** through the upper side of the upper mold. These air vents **15a** and **15b** are **15** connected to a vacuum pump **3**. Optionally, the air vents **15a** and **15b** may be utilized as simple ducts for spent gas instead of being connected to the vacuum pump **3**.

A sprue (through hole) **21** communicating with the runner **13** mentioned above is formed at a pertinent position of the lower mold **20**. Underneath the sprue **21** is formed a depression **22** which is shaped to conform with a cylindrical raw material accommodating part **32** constituting itself an upper part of a melting vessel **30**. To the sprue **21** of the lower mold **20**, an inlet ring or sprue bush **23** made of such insulating material as a ceramic substance or a metal of small thermal conductivity is fitted. The sprue **21** (the inner wall of the sprue bush **23**) is diverged downwardly to form a truncated cone space so that the molten alloy is smoothly introduced into the molding cavity.

Further in the upper mold **11**, a vertical through hole **16** is formed above the upper part of the sprue **21**. In the through hole **16**, a rodlike cutting member **17** having a cutting edge **18** formed along the circular edge of the lower end thereof is disposed so as to be vertically reciprocated in the direction of the sprue **21**. The cutting member **17** is actuated by a hydraulic cylinder (or a pneumatic cylinder) disposed thereover and not shown in the diagram. A closing member or closing rod **19** is interposed between the lower end of the cutting member **17** and the runner **13**. This closing member **19**, as clearly shown in FIG. 2, has ridges **24** raised from the opposite side faces thereof and meshed with grooves **26** in a hole **25** formed in the horizontal direction in the upper mold so that the closing member **19** is slidable in the perpendicular direction relative to the direction of the motion of the cutting member **17** (in the bearings of the diagram, in the perpendicular direction to the face of paper). The closing member **19**, during the introduction of the molten alloy, has the leading end part thereof thrust into the through hole **16** so as to prevent the molten alloy from being poured into the through hole **16**. After the molten alloy has been poured and solidified, the closing member **19** retracts to the extent of opening the lower part of the through hole **16** and causing the cutting edge **18** at the lower end of the cutting member **17** to protrude as far as the sprue **21**. The closing member **19** is preferred to be made of such insulating material as mentioned above.

While the forced cooling casting mold **10** can be made of such metallic material as copper, copper alloy, cemented carbide or superalloy, it is preferred to be made of such material as copper or copper alloy which has a large thermal capacity and high thermal conductivity for the purpose of heightening the cooling rate of the molten alloy poured into the cavities **12a** and **12b**. The upper mold **11** has disposed therein such a flow channel as allow flow of a cooling medium like cooling water or cooling gas. The flow channel is omitted from the drawing by reason of limited space.

The melting vessel **30** is provided in the upper part of a main body **31** thereof with the cylindrical raw material accommodating part or pot **32** and is disposed directly below the sprue **21** of the lower mold **20** so as to be reciprocated vertically. In a raw material accommodating hole **33** of the raw material accommodating part **32**, a molten metal transferring member or piston **34** having nearly the same diameter as the raw material accommodating hole **33** is slidably disposed. The molten metal transferring member **34** is vertically moved by a plunger **35** of a hydraulic cylinder (or pneumatic cylinder) not shown in the diagram. An induction coil **36** as a heat source is disposed so as to encircle the raw material accommodating part **32** of the melting vessel **30**. As the heat source, any arbitrary means such as one resorting to the phenomenon of resistance heating may be adopted besides the high-frequency induction heating. The material of the raw material accommodating part **32** and that of the molten metal transferring member **34** are preferred to be such heat-resistant material as ceramics or metallic materials coated with a heat-resistant film.

For the purpose of preventing the molten metal from forming an oxide film, the forced cooling casting mold **10** and the melting vessel **30** are disposed in a chamber **1**. The apparatus in its entirety is maintained in a vacuum by actuating a vacuum pump **2** which is connected to the interior of the chamber **1**. Otherwise, an inert gas such as Ar gas is introduced into the chamber **1** to establish an atmosphere of the inert gas and enclose the relevant parts with the atmosphere.

In preparation for the production of a tube of amorphous alloy, first the alloying raw material **A** of such a composition capable of yielding an amorphous alloy as mentioned above is placed in the empty space overlying the molten metal transferring member **34** inside the raw material accommodating part **32** while the melting vessel **30** is held in a state separated downwardly from the forced cooling casting mold **10**. The alloying raw material **A** to be used may be in any of the popular forms such as rods, pellets, and minute particles.

Subsequently, the vacuum pump **2** is actuated to reduce the inner pressure of the chamber **1** or the Ar gas is introduced to create an inert atmosphere. Thereafter, the induction coil **36** is excited to heat the alloying raw material **A** rapidly. After the fusion of the alloying raw material **A** has been confirmed by detecting the temperature of the molten metal, the induction coil **36** is demagnetized and the melting vessel **30** is elevated until the upper end thereof is inserted in the depression **22** of the lower mold **20**. At this time, the closing member **19** thrusts into the lower part of the through hole **16** and the communication between the through hole **16** and the runner **13** is blocked.

Then, the vacuum pump **3** is actuated to lower the pressure in the cavities **12a** and **12b** of the forced cooling casting mold **10** below the pressure in the chamber **1**. Thereafter, the hydraulic cylinder (not shown) is actuated to effect rapid elevation of the molten metal transferring member **34** and injection of the molten metal **A'** through the sprue **21** of the casting mold **10** as illustrated in FIG. 2. The injected molten metal **A'** is advanced through the runner **13**, introduced into the cavities **12a** and **12b**, and compressed and rapidly solidified therein. In this case, the cooling rate exceeding  $10^3$  K/s can be obtained by suitably setting the injection temperature, the injection speed, etc.

After the molten metal charged in the cavities has been solidified, the closing member **19** is retracted to open the lower part of the through hole **16** as illustrated in FIG. 3 and then the hydraulic cylinder (not shown) is actuated to effect

rapid downward thrust of the cutting member 17 and consequent severance of the runner part of a solidified material A" by the cutting edge 18 thereof as illustrated in FIG. 4. At this time, the solidified material A" lodged in the peripheral part of the sprue 21 can be easily cut by the cutting member 17 because it is made to cool at a lowered rate and is consequently crystallized and embrittled owing to the use of an insulating material for the sprue bush 23 and the closing member 19. A solidified material A" in the severed portion of the sprue 21 is dropped into the raw material accommodating part 32 of the melting vessel 30 and put to reuse.

Then, after the melting vessel 30 has been returned to the home position thereof as indicated by an imaginary line in FIG. 4 and the cutting member 17 has been elevated, the leading end part of the closing member 19 is advanced until the lower part of the through hole 16 is closed.

Thereafter, the upper mold 11 and the lower mold 20 are separated from each other and the cast article is extracted from the interior of the forced cooling casting mold 10 to complete the first round of the production step.

In the next round of the production step, the melting vessel 30 is replenished, as occasion demands, with the alloying raw material  $\Delta$  and then, similarly in the step described above, the alloying raw material  $\Delta$  is melted, the melting vessel 30 is elevated until the upper end of the raw material accommodating part 32 is inserted in the depression 22 of the lower mold 20, and the molten metal transferring member 34 is rapidly elevated as illustrated in FIG. 5 to effect the second round of injection. Thereafter, the second round of production step is completed by repeating the same procedure as described above. The step of the procedure described above is then repeated.

The shape of the cast article produced by the method described above is illustrated in FIG. 6 and FIG. 7. Tubes having a smooth surface faithfully reproducing the cavity surface of the casting mold are obtained by severing runner parts 42a and 42b from cylindrical parts 41a and 41b of a cast article 40 and grinding the cut faces of the cylindrical parts 41a and 41b remaining after the severance. Though the runner parts 42a and 42b and a sprue part 43 of the cast article 40 have been already severed by the cutting member 17 as described above, they are depicted in a connected state in FIG. 6 and FIG. 7 to facilitate comprehension of the shapes of the molding cavities 12a and 12b, and runners 13 and semicircular parts 14a and 14b thereof of the forced cooling casting mold 10 illustrated in FIG. 1.

The method described above allows manufacture of tubes which have a dimensional accuracy,  $L, \pm 0.0005$  to  $\pm 0.001$  mm and a surface accuracy 0.2–0.4  $\mu\text{m}$ .

The apparatus, as described above with reference to FIG. 1, uses a forced cooling casting mold 10 forming a pair of molding cavities 12a and 12b and manufactures two products by a single step. It is naturally permissible to use a forced cooling casting mold forming three or more cavities and manufactures that many products. One example of such manufacture of a multiplicity of cast articles is illustrated in FIG. 8.

FIG. 8 depicts a cast article 40a having four cylindrical parts 41a, 41b, 41c, and 41d joined to runner parts 42a and 42b. A larger number of cast articles can be manufactured by a single step, when necessary, by having as many molding cavities disposed around the sprue 21 of the forced cooling casting mold 10.

The high-pressure mold casting method described above allows a casting pressure up to about 100 MPa and an injection speed up to about several m/s and enjoys the following advantages.

(1) The charging of the forced cooling casting mold with the molten metal completes within several milliseconds and this quick charging adds greatly to the action of rapid cooling.

(2) The highly close contact of the molten metal to the forced cooling casting mold adds to the speed of cooling and allows precision molding of molten metal as well.

(3) Such faults as shrinkage cavities possibly occurring during the shrinkage of a cast article due to solidification can be allayed.

(4) The method allows manufacture of a formed article in a complicated or delicate shape.

(5) The method permits smooth casting of a highly viscous molten metal.

FIG. 9 depicts schematically the construction of one example of the apparatus for producing a toothed wheel of amorphous alloy according to the method of the present invention.

In the apparatus illustrated in FIG. 9, a forced cooling casting mold 10a is composed of an upper mold 11a, a lower mold 20a, and one pair of laterally opposite molds 27 and 28. This casting mold 10a is different from the forced cooling casting mold 10 illustrated in FIG. 1 in respect that one pair of product molding cavities 29a and 29b conforming with the contour of a produced toothed wheel are interposed respectively between the upper and lower molds 11a and 20a and the left mold 27 and the right mold 28. Since such component parts of the casting mold as a sprue 21a, a sprue bush 23a surrounding the sprue 21a, a cutting member 17a disposed vertically movably thereabove, and a closing member 19a disposed thereunder are identical in material and structure to the corresponding component parts of the forced cooling casting mold illustrated in FIG. 1, their description will be omitted herein.

A melting vessel adapted to reciprocate freely in the vertical direction is disposed below the sprue 21a of the forced cooling casting mold 10a. Since this melting vessel is identical in construction with that of the apparatus illustrated in FIG. 1, the illustration thereof is omitted herein. The forced cooling casting mold 10a and the melting vessel are disposed in the chamber 1.

Since the process of production by the use of the apparatus shown in FIG. 9 is similar in the production by the apparatus illustrated in FIG. 1, therefore, the description thereof is omitted herein.

Use of the forced cooling casting mold 10a illustrated in FIG. 9 allows manufacture by casting of such a toothed wheel 45 of amorphous alloy as illustrated in FIG. 10.

FIG. 11 depicts an example of the apparatus for producing a tube of amorphous alloy by another method of the present invention.

This apparatus has a construction such that a lower mold 51 and an upper mold 60 of a forced cooling casting mold 50 are substantially reciprocal in layout to the upper mold 11 and the lower mold 20 of the forced cooling casting mold 10 illustrated in FIG. 1. Specifically, the lower mold 51 has a pair of molding cavities 52a and 52b for defining the outside dimension of the tube. Then, in these cavities 52a and 52b, cores 65a and 65b for defining the inside dimension of the tube are disposed respectively. These cores 65a and 65b are raised from the lower side of the upper mold 60. The cavities 52a and 52b intercommunicate through the medium of a runner 53 such that the molten metal flows through the leading end of such parts 54a and 54b of the runner 53 as half encircle the peripheries of the cavities 52a and 52b at a

prescribed distance into the cavities **52a** and **52b**. The cylindrical parts of molten metal transferring members **55a** and **55b** which are adapted to reciprocate freely in the vertical direction are disposed slidably in the empty spaces between the cavities **52a** and **52b** and the cores **65a** and **65b**. Inside a vertical through hole **56** formed in the lower part of the runner **53**, a rodlike cutting member **57** having a cutting edge **58** formed along the periphery of the upper end thereof is disposed movably toward a sprue **61**. Further, between the upper end of the cutting member **57** and the runner **53**, a closing member **59** is slidably disposed perpendicularly to the direction of movement of the cutting member **57**. The structures of the cutting member **57** and the closing member **59** and the operating mechanisms of the molten metal transferring members **55a** and **55b**, the cutting member **57**, and the closing member **59** are similar to those in the apparatus illustrated in FIG. 1, excepting that they are reciprocal in layout.

The sprue (through hole) **61** communicating with the runner **53** mentioned above is formed at a pertinent position of the upper mold **60** and a depression **62** conforming with the lower end part of a cylindrical melting vessel **70** is formed in the upper edge part of the sprue **61**. A sprue bush **63** made of an insulating material and having a diverging inner diameter is fitted to the sprue **61** of the upper mold **60** and a closing member **64** made of an insulating material and having the same structure as the closing member **59** mentioned above is disposed in the lower end part of the sprue bush **63** in such a manner as to be slidably moved in a direction perpendicular to the direction of the axial line of the sprue **61** (the direction of movement of the cutting member **57**).

The melting vessel **70** is a cylindrical container and is disposed directly above the sprue **61** of the upper mold **60** in such a manner as to be freely reciprocated in the vertical direction. It is encircled with an induction coil **71**.

The forced cooling casting mold **50** and the melting vessel **70** are disposed within the chamber **1** similarly in the apparatus shown in FIG. 1.

In preparation for the production of a tube by the use of the apparatus shown in FIG. 11, first the melting vessel **70** is lowered. Now, the melting vessel **70**, with the lower end thereof fitted in the depression **62** of the upper mold **60** of

sprue **61** via the runner **53** into the cavities **52a** and **52b** and, meanwhile, a pressurized gas is introduced into the melting vessel **70** to press the molten metal.

After the molten metal filling the cavities has been solidified, the melting vessel **70** is elevated and, similarly in the apparatus illustrated in FIG. 1, the closing member **59** is retracted to open the upper part of the through hole **56**, then the hydraulic cylinder (not shown) is actuated to effect rapid upward thrust of the cutting member **57**, and the cutting edge **58** of the cutting member **57** is caused to sever the runner part of the solidified material. At this time, the solidified material lodged in the sprue **61** can be easily cut by the cutting member **57** because it is made to cool at a lowered rate and is consequently crystallized and embrittled owing to the use of an insulating material for the sprue bush **63** and the closing member **59**. The solidified material in the portion of the sprue **61** severed from the cast product is removed from the upper mold and put to reuse.

After the cutting member **57** has lowered subsequently, the leading end parts of the closing member **59** and **64** advance and respectively close the upper part of the through hole **56** and the lower part of the sprue **61**.

Thereafter, the upper mold **60** and the lower mold **51** are separated and the molten metal transferring members **55a** and **55b** are elevated to eject the cast article from the forced cooling casting mold **50** and complete the first round of the step of production.

Now, the mechanical properties of the aforementioned amorphous alloys will be described below with reference to the results of the test therefor. The specimens were manufactured as follows:

Various alloys including  $Zr_{60}Al_{15}Co_{2.5}Ni_{7.5}Cu_{15}$  and shown in the following table were manufactured by melting relevant component metals. They were each placed in a quartz crucible and melted thoroughly by high-frequency induction heating. The melt was injected under a gaseous pressure of  $2 \text{ kgf/cm}^2$  through a slender hole formed in the lower part of the crucible into a copper mold provided with a cylindrical cavity, 2 mm in diameter and 30 mm in length, and kept at room temperature to obtain a rod-like specimen for the determination of mechanical properties. The results of this determination are shown in the table.

TABLE

| Alloy used                              | $\frac{\alpha}{10^{-5}/\text{K}}$ |                        |                       |         |             |        |        |
|-----------------------------------------|-----------------------------------|------------------------|-----------------------|---------|-------------|--------|--------|
|                                         | Tensile strength (MPa)            | Bending strength (MPa) | (room temperature-Tg) | E (GPa) | Hardness Hv | Tg (K) | Tx (K) |
| $Zr_{67}Cu_{33}$                        | 1,880                             | 3,520                  | 0.8                   | 99      | 540         | 603    | 669    |
| $Zr_{65}Al_{7.5}Cu_{27.5}$              | 1,450                             | 2,710                  | 0.8                   | 93      | 420         | 622    | 732    |
| $Zr_{65}Al_{7.5}N_{10}Cu_{17.5}$        | 1,480                             | 2,770                  | 0.9                   | 92      | 430         | 630    | 736    |
| $Zr_{60}Al_{15}Co_{2.5}Ni_{7.5}Cu_{15}$ | 1,590                             | 2,970                  | 1.0                   | 91      | 460         | 652    | 768    |

the forced cooling casting mold **50**, is charged with the alloying raw material  $\Delta$  of a composition capable of yielding such amorphous alloy as mentioned above. Then, the induction coil **71** is excited to heat the alloying raw material  $\Delta$  rapidly. After the alloying raw material  $\Delta$  has been melted, the induction coil **71** is demagnetized, the closing member **64** is retracted to open the lower part of the sprue **61**, the molten metal transferring members **55a** and **55b** are rapidly lowered to generate negative pressure in the molding cavities **52a** and **52b**, the molten metal is aspirated from the

It is clearly noted from the table that the produced amorphous alloy materials showed such magnitudes of bending strength as notably surpass the magnitude (about 1,000 MPa) of the partially stabilized zirconia heretofore adopted as the material for a formed ceramic article, such magnitudes of Young's modulus as approximate one half, and such magnitudes of hardness as approximate one third thereof, indicating that these alloy materials were vested with properties necessary as the material for various formed articles.

## 13

According to the present invention, as described above, a formed article of amorphous alloy satisfying a predetermined shape, dimensional accuracy, and surface quality despite complexity or delicateness of shape can be manufactured with high productivity at a low cost owing to the combined use of a technique based on the metal mold casting process with the amorphous alloys exhibiting a glass transition region. Further, since the amorphous alloy to be used for the present invention excels in strength, toughness, and resistance to corrosion, various precision formed articles manufactured from this amorphous alloy withstand long service without readily sustaining abrasion, deformation, chipping, or other similar defects.

While certain specific embodiments have been disclosed herein, the invention may be embodied in other specific forms without departing from the spirit or essential characteristics thereof. The described embodiments are therefore to be considered in all respects as illustrative and not restrictive, the scope of the invention being indicated by the appended claims rather than by the foregoing description and all changes which come within the meaning and range of equivalency of the claims are, therefore, intended to be embraced therein.

What is claimed is:

1. A method for the production of a formed article of amorphous alloy, comprising the steps of:

providing a melting vessel having an upper open end and a forced cooling casting mold provided with at least one molding cavity and cooperating with said melting vessel;

melting an alloying material capable of yielding an amorphous alloy in said melting vessel;

forcibly transferring the resultant molten alloy into the molding cavity of said forced cooling casting mold via a sprue thereof and meanwhile exerting pressure on the molten alloy;

rapidly cooling and solidifying said molten alloy in said forced cooling casting mold thereby conferring amorphousness on the alloy and meanwhile gradually cooling and solidifying the molten alloy in the part of said sprue of said forced cooling casting mold thereby crystallizing the alloy in said part;

cutting the part which has been embrittled by said crystallization; and

separating said melting vessel from said forced cooling casting mold to obtain a formed article of an alloy containing an amorphous phase.

## 14

2. The method according to claim 1, wherein said melting vessel is provided with a molten metal transferring member disposed movably in said melting vessel and said molten metal transferring member is caused to transfer forcibly the molten alloy in said melting vessel into the molding cavity of said forced cooling casting mold and meanwhile exert pressure on said molten alloy filling the molding cavity of said forced cooling casting mold.

3. The method according to claim 1, wherein said forced cooling casting mold is provided with a molten metal transferring member disposed movably in said forced cooling casting mold and said molten metal transferring member is moved so as to generate negative pressure in said molding cavity and effect forced transfer of said molten alloy into said molding cavity.

4. The method according to claim 3, wherein a gas pressure is added to the melting vessel during forced transfer of said molten alloy into said molding cavity.

5. The method according to claim 3, wherein said molten metal transferring member is possessed of a cross section conforming with the contour of said molding cavity of said forced cooling casting mold and slidably disposed in said molding cavity.

6. The method according to claim 1, wherein said alloying material capable of yielding said amorphous alloy is melted by high-frequency induction heating or resistance heating.

7. The method according to claim 1, wherein said forced cooling casting mold is a water-cooled casting mold or gas-cooled casting mold.

8. The method according to claim 1, wherein said alloying material is an alloy having a composition represented by the following general formula and endowed with an ability to yield an amorphous alloy having a glass transition region of a temperature width of not less than 30 K:



wherein X represents either or both of two elements, Zr and Hf, M represents at least one element selected from the group consisting of Mn, Fe, Co, Ni, and Cu, and a, b, and c represent such atomic percentages as respectively satisfy  $25 \leq a \leq 85$ ,  $5 \leq b \leq 70$ , and  $0 < c \leq 35$ , and said amorphous alloy contains an amorphous phase in a volumetric ratio of at least 50%.

9. The method according to claim 1, wherein said melting of said alloying material in said melting vessel is carried out in a vacuum or under an atmosphere of inert gas.

\* \* \* \* \*